

# UNITED STATES PATENT OFFICE.

FRANK A. FAHRENWALD, OF CLEVELAND HEIGHTS, OHIO.

## FIREARM AND ALLOY FOR MAKING SAME.

1,346,191.

Specification of Letters Patent.

Patented July 13, 1920.

No Drawing.

Application filed December 15, 1919. Serial No. 345,083.

To all whom it may concern:

Be it known that I, FRANK A. FAHRENWALD, a citizen of the United States, residing at Cleveland Heights, in the county of Cuyahoga and State of Ohio, have invented a certain new and useful Improvement in Firearms and Alloys for Making Same, of which the following is a full, clear, and exact description.

10 This invention relates to firearms and ordnance and has for its object a provision of metallic alloy for use in construction of the same which shall be more resistant to corrosion by the combustion products of the 15 explosives as well as less effected by atmospheric conditions and salt solutions (such as sea water or perspiration) than any of the materials now in use for the purpose; which shall be at least as easily man- 20 ufactured as the steels at present employed, which shall be at least equally resistant with steel to mechanical erosion and less subject than steel to becoming fouled by the material of the bullets or projectiles em- 25 ployed; and which shall not be unduly high in intrinsic value.

Practically the only substance now in use for the barrels of firearms and ordnance is some kind of a steel, in other words con- 30 tains a considerable percentage of carbon in the form of iron carbide dissolved in an excess of iron. This is sometimes modified by the presence of a very small percentage of nickel, vanadium, tungsten, etc., but the 35 essential characteristics are those of steel, which include the capacity of becoming hardened by heating and quenching together with high susceptibility to the corrosive effect of powder gases, powder re- 40 sidues, salt solutions and other rusting conditions. Furthermore such carbides are seldom disseminated with perfect uniformity throughout the mass of material, and be- sides, owing to their susceptibility to tem- 45 perature influences, it is seldom that all parts are given the same degree of hard- ness or temper which produces an inequality of strain within the material. The con- sequence is that when a barrel of steel 50 is bored, the effect of the perforation is to release this strain unequally in different parts of the barrel which therefore automatic- 55 ically bends in one direction or the other as a result of the boring operation alone and hence requires a careful straightening op-

eration which is a task fit only for the most expert of workmen. Furthermore such a barrel when heated by repeated firing always becomes warped and thus produces a deflection of the bullet depending upon the temperature.

According to my invention I avoid the faults due to these characteristics of steel by reducing the carbon content to the lowest possible extent, and secure the necessary 60 hardness and toughness of the metal by the use of some substance other than carbon which shall have the added capability of shielding the fundamental metal against corrosive action. Owing to its cheapness 65 and availability I prefer to employ iron as the fundamental metal, although other metals of the iron group can equally be employed, and in fact serve the purpose to a degree even superior to iron, although the 70 iron-base-alloy is sufficient for every practical purpose. The two basic protective metals for use with iron are chromium and nickel. They may be used either separately, or together, either with or without 75 other substances. An alloy of iron with 10% of either of the metals, chromium or nickel, possesses resistivity to corroding influences far superior to anything heretofore used in firearms as also does an alloy 80 of iron combined with both chromium and nickel up to this percentage, the latter occurring in any desired proportion relatively to each other.

The effect of carbon on these alloys is to 85 harden the same to a much greater extent than in the case of an alloy not containing these ingredients and as a result it is necessary to keep the amount of carbon very low. .2 of 1% appears to be about the up- 90 permost desirable limit of carbon, and with the higher percentages of either or both of the metals, nickel or chromium, the carbon 95 ought to be retained below about .1 of 1%. The necessary hardness in the alloy is se- 100 cured by either, nickel or chromium in amounts of 10% or upward and these amounts also afford marked chemical resistivity. The upper limit of chromium is about 25% since above this amount the al- 105 loy becomes too hard for convenient fabri- cating, there is no limit upon the proportion of nickel other than economic considera- tions.

These alloys can readily be made in the 110

electric furnace by the use of pure materials and can be melted, cast, forged, drilled, rifled and otherwise fabricated with the same facility as steel. Barrels made of the same 5 do not require to be straightened after boring as in the case of steel and do not show any tendency to deflection upon heating. The surface of the metal tends to become smoother and more polished the more frequently it is fired and offers far less tendency than steel barrels to become fouled or eroded by the material of the projectiles; barrels containing upward of about 10% of 10 chromium are highly immune to gasses and residues of all explosives, even when left uncleaned for long periods, while chromium alloys above about 12% are completely immune. Barrels of iron alloyed with 30% or more of 15 nickel will withstand severe neglect and alloys containing 15% of nickel together with 10% of chromium are entirely immuned. 20 10% of nickel is not enough to confer high immunity for barrel use, but produces an alloy which is excellent for breech blocks, actions, etc., since it is markedly resistant to 25 atmospheric influences.

There are other metals than nickel or chromium which will exert a protective effect upon iron together with the hardening 30 effect made necessary by the reduction in carbon content, but suffer the disadvantage either of requiring undue amounts to confer equal chemical resistivity or exert injurious effects upon the physical properties 35 when employed to a sufficient extent to produce by themselves the desired protection effect. Cobalt is the full equivalent of nickel in this relation but is of less practical value because of its comparatively high cost. 40 Small quantities of vanadium, titanium, or manganese are very desirable for use as

scavengers and the presence of small amounts of vanadium or manganese in the finished alloy is an advantage but titanium or zirconium, if used as scavengers should 45 be restricted to the exact amount which will be eliminated in process unless carbon and silicon are substantially entirely eliminated. These substances are to be used in addition to the nickel or chromium and not in substitution therefor, wherefore I consider the preferable alloy to be essentially that of iron with either or both nickel and (or) chromium, the highest limit of chromium being about 25 and the highest limit of 50 iron about 90, and the lowest limit of nickel or chromium or some combination of the two being about 10%.

While I have suggested this principally in connection with the barrels of firearms I do 60 not exclude its use for breech blocks, firing mechanisms, etc., which parts are also subjected to some extent to powder fumes and residues and to an equal or greater extent 65 to atmospheric and salt conditions.

Having thus described my invention, what I claim is:

1. A firearm barrel made of an alloy containing iron combined with at least about 70 thirty per cent. of one or more other metals of the iron group.

2. A firearm barrel made of an alloy containing one or more iron group metals alloyed with such an amount of chromium that the total amount of non-ferrous metal 75 in the alloy shall constitute about twenty-five per cent. of the whole, and the chromium constituting at least about five per cent. of the whole.

In testimony whereof, I hereunto affix my 80 signature.

FRANK A. FAHRENWALD.